

## UNITED STATES PATENT OFFICE

2,212,826

## REFRIGERATING SYSTEM

Frederick B. Downing, Penns Grove, N. J., and William Henry Markwood, Jr., Fairville, Pa., assignors to Kinetic Chemicals, Inc., Wilmington, Del., a corporation of Delaware

No Drawing. Application October 25, 1939,  
Serial No. 301,228

5 Claims. (Cl. 62—178)

A. This invention relates to processes of refrigeration for systems containing iron and copper parts and utilizing a halogenated hydrocarbon refrigerant.

B. In refrigerating systems which use halogenated hydrocarbons such as methyl chloride and dichlorodifluoromethane as refrigerants a phenomenon is observed which is called copper plating. Parts of the system which are made of non-cuprous metals, notably the moving parts such as pistons and valves, become coated with a layer of copper. This coating may proceed to the point where the efficiency of the apparatus is materially decreased or to the point where the apparatus may be unable to function. In these systems mineral oil is generally used as a lubricant and it has been observed that much of the plating occurs on the portions of the apparatus which need lubrication or which are in constant contact with the lubricant. This has led to the theory that copper from the tubes or other portions of system, which are formed of that metal or of alloys thereof, is dissolved or suspended in the lubricant, or in mixtures of the lubricant and refrigerant, and deposited on those parts.

C. Regardless of the manner in which it occurs, however, it is an object of this invention to inhibit copper plating in refrigerating systems of the type described.

D. The objects of the invention are accomplished, generally speaking, by including in the system a small amount of picolinic acid. The picolinic acid can be added with successful results to the lubricating oil which is used in the system.

E. Although the manner in which picolinic acid functions as an inhibitor of copper-plating is not clearly understood, it is thought that the copper in the parts of refrigeration systems constructed of this metal, forms a chelate compound with picolinic acid producing a relatively insoluble, adherent film on the metallic surface. The plating of the copper from the relatively small amount of the complex that may be in solution is probably prevented by the formation of a similar chelate iron complex on the iron and steel surfaces where the plating would normally occur in the absence of picolinic acid. However, the applicants do not wish to be bound by any particular theory of operation.

F. The following example illustrates, but does not limit the invention; the picolinic acid being

used in any amount which is necessary to produce optimum results.

*Example*

Of picolinic acid .1% by weight calculated on the amount of lubricant present in the system was added to a refrigerating system containing methyl chloride refrigerant and a mineral oil lubricant. The system was operated for a period of time which is sufficient to produce objectionable copper plating in systems not containing picolinic acid and it was found that copper plating had been entirely prevented. It has been demonstrated that additions of picolinic acid from 0.05% to 1.0% based on the weight of the lubricant employed are sufficient to inhibit or to totally prevent copper plating.

G. Although copper plating has occurred in household and some industrial refrigerating units, it has been more bothersome in large units employing heavy duty compressors. This has to some extent reduced the application of halogenated hydrocarbon refrigerants in the heavy duty field. By this invention the objection to halogenated hydrocarbon refrigerants in the heavy duty field is removed.

H. As many apparently widely different embodiments of this invention may be made without departing from the spirit and scope thereof, it is to be understood that we do not limit ourselves to the specific embodiments thereof except as defined in the appended claims.

We claim:

1. A process of refrigeration which comprises condensing and evaporating a halogenated hydrocarbon in the presence of a mineral oil containing picolinic acid.

2. The process of claim 1 in which the mineral oil contains from 0.05% to 0.1% of picolinic acid.

3. The process of claim 1 in which the mineral lubricating oil contains about 0.1% of picolinic acid.

4. A refrigerating system containing iron parts, copper parts, a halogenated hydrocarbon refrigerant, a lubricating oil, and picolinic acid.

5. The method of inhibiting copper plating in a refrigerating system containing a halogenated hydrocarbon refrigerant which comprises adding picolinic acid to the system.

FREDERICK B. DOWNING.  
WILLIAM H. MARKWOOD, JR.